

Dec. 29, 1936.

L. C. BEARD, JR

2,065,551

METHOD OF PREPARING LUBRICANTS

Filed March 14, 1934



*Luke C Beard Jr.*  
INVENTOR

BY  
*Myron J. Dubland*  
ATTORNEY

## UNITED STATES PATENT OFFICE

2,065,551

## METHOD OF PREPARING LUBRICANTS

Leslie C. Beard, Jr., Brooklyn, N. Y., assignor to  
Socony-Vacuum Oil Company, Incorporated, a  
corporation of New York

Application March 14, 1934, Serial No. 715,470

4 Claims. (Cl. 196—13)

This invention has to do with the preparation of lubricating oils of good quality from sources not hitherto used, such as residues from the cracking of gas oils under heat and pressure, 5 and the like.

It has long been known that in the cracking under heat and pressure of gas oils and the like to produce gasoline, that some of the oil seems to react in the reverse direction. That is, when a 10 charging stock containing initially no material heavier or lighter than gas oil is subjected to controlled conditions of heat and pressure for the production of gasoline, a considerable portion of the charge is converted into materials of heavier 15 nature. It has been recognized that certain fractions of these heavier products had the properties of lubricants at ordinary temperatures, and it has been proposed to separate these "lubricant" fractions and use them as such. Experience with 20 these products, prepared by simple distillation from cracking residues and refined by the current methods has been disappointing. The oils so prepared have a much greater tendency toward oxidation and sludging than ordinary oils 25 of the same general characteristics, and of more importance, lose viscosity with increase of temperature much more rapidly than most of the more rapidly thinning normal oils. Additionally such oils have an abnormally high gravity for a given viscosity. All of these qualities have militated against the adoption and widespread use 30 of such oils. Attempts have been made to cover or alter these properties by blending such products with other oils and by combining them with other materials, such as sulphur, for instance, 35 but without notable success.

I have found that by properly refining these oils, lubricants can be made which compare favorably in all respects with normally produced lubricants now on the market.

It has therefore been an object of this invention to prepare a lubricant of normal characteristics from sources now deemed incapable of yielding such an oil, to devise a process whereby 45 that lubricant can be recovered and refined, to develop methods whereby the cracking of gas oils can be caused to yield good lubricants as well as gasoline, and such other objects and advantages as may hereinafter appear.

To assist in the further discussion, reference 50 is made to that property of lubricants known as "viscosity index", and developed by Dean and Davis, Chemical and Metallurgical Engineering, vol. 36, page 618. In brief, viscosity index is 55 a measure of the tendency of a lubricant to become less viscous at high temperatures, as measured by the viscosities at 100° F. and 210° F. respectively, as related to certain oils used as standards. The index so calculated for present day lubricants derived from Pennsylvania grade crude

is approximately 100, that for most grades of Mid-Continent base lubricants range from 60 to 80, and for some Texas Gulf Coastal base lubricants range from zero to 20. The lower the viscosity index, the greater the rapidity with which the oil loses viscosity on heating. The scale is arbitrarily fixed.

A further criterion of value is that known as the viscosity-gravity constant. This was developed by Hill and Coates, Industrial and Engineering Chemistry, 1928, page 641, the equation being:

Viscosity-gravity constant =  
Specific gravity  $-0.24 - 0.022 \log_{10} (\text{Vis} @ 210 - 35)$

.755 15  
The viscosity-gravity constant of present day lubricants of Pennsylvania origin range from approximately .800 to .830, of Mid-Continent lubricants from .830 to .870, and of California and Gulf Coastal oils from .870 to .890. This 20 classification is not entirely rigid, some oils otherwise having properties consistent with their source falling out of place in the above rough classification.

The process of my invention may be very briefly described as separating from a pressure tar, by distillation, the fraction containing ingredients capable of being refined into acceptable lubricants, separating unacceptable lubricants from the distillate fraction by suitable methods, and finishing the remaining portion of the distillate fraction into commercially acceptable lubricants.

The essential features of my process may be noted by reference to the drawing attached to this specification, which shows in outline form 35 the sequence of steps herein disclosed.

As an example of my process, I may cite the following:

A gas oil of normal characteristics, containing no lubricant fractions, but composed of fractions much less viscous than lubricants, was charged to a Cross cracking still, and subjected to the usual conditions of operation therein. From this cracking process a tar was recovered, which had the following characteristics:

|                       |                   |
|-----------------------|-------------------|
| Gravity               | 12.8° A. P. I.    |
| Viscosity             | 19" Saybolt furol |
| Initial boiling point | 331° F.           |
| 70% over at           | 705° F.           |

This is a typical cracking still tar. The characteristics of such products will vary slightly, depending upon the details of the cracking operation, but, in general, any cracking process operating upon gas oil will produce tar comparable substantially to the typical tar above set forth, or containing a substantial portion of products similar to products which may be separated from the above tar.

The above tar was then charged to a vacuum 60

still and distilled at an absolute pressure of 5 mm. mercury. The condensate fraction between 56% over and 80% over, inclusive, was collected, and found to have the following properties:

|                         |                         |
|-------------------------|-------------------------|
| 5 Gravity               | 10.3° A. P. I.          |
| Flash C. O. C.          | 445° F.                 |
| Fire C. O. C.           | 520° F.                 |
| Pour point              | 35° F.                  |
| Viscosity at 100° F.    | 1032" Saybolt universal |
| 10 Viscosity at 130° F. | 343" Saybolt universal  |
| Viscosity at 210° F.    | 65" Saybolt universal   |
| Viscosity index         | Minus 12                |
| Color                   | Dark green              |
| Conradson carbon        | 1.56%                   |
| 15 Sulphur              | 0.79%                   |

I have found that by subjecting this oil to certain methods of refining, there may be isolated from it an acceptable lubricant. The refining methods capable of performing this operation are 20 those methods broadly known as selective solvent refining methods.

The general aim of these selective solvent methods is to increase the viscosity index of the oil treated by separating from it ingredients of low resistance to loss of viscosity with rise in temperature. 25 Among various agents proposed for this purpose there may be named nitrobenzene, benzonitrile, phenol, furfural, acrolein, and crotonaldehyde, dichloroethyl ether, (known as "chlorex"), mixtures of liquid sulphur dioxide and benzol, liquid sulphur dioxide, and similar solvents. These 30 above named reagents act as selective solvents for the ingredients of low viscosity index originally present in the oil, and remove them as an extract. It is also possible to use liquid propane, either pure or mixed with small percentages of butane, etc. for this purpose, this reagent acting 35 as a selective solvent for the ingredients of high viscosity index. Other processes of this type propose to use simultaneously two counter-current solvent streams, such as for instance cresol for the selective solution of ingredients of low viscosity index, and liquid propane for the selective 40 solution of ingredients of high viscosity index, as in Tuttle, U. S. Patent No. 1,912,349. The functional operation of all of these processes are somewhat similar, the actual details of operation are 45 characteristic of each process, and of the stock being treated, and all are directed to the same 50 end.

In the present example, I have treated the above mentioned vacuum distillate fraction of pressure tar with liquid sulphur dioxide, using 55 four batch extractions at 16° F., and each time treating the oil with an amount of liquid sulphur dioxide equal in volume to 50% of the oil being treated. From the distillate I recovered approximately 40% of a refined oil having the following 60 properties:

|                            |                        |
|----------------------------|------------------------|
| Gravity                    | 21.3° A. P. I.         |
| Flash C. O. C.             | 425° F.                |
| Fire C. O. C.              | 490° F.                |
| Pour point                 | 65° F.                 |
| Viscosity at 100° F.       | 347" Saybolt universal |
| Viscosity at 130° F.       | 160" Saybolt universal |
| Viscosity at 210° F.       | 52" Saybolt universal  |
| Viscosity index            | 71                     |
| Color                      | Dark 8                 |
| 70 Conradson carbon        | 0.25%                  |
| Sulphur                    | 0.48%                  |
| Viscosity gravity constant | .875                   |

With the exception of pour point, this is to all respects a good lubricant, capable of comparison

with the greater volume of lubricants on today's markets. To reduce the pour point, I dewaxed this oil, yielding a finished oil of the following tests:

|                            |                        |
|----------------------------|------------------------|
| Gravity                    | 20.5° A. P. I.         |
| Flash C. O. C.             | 435° F.                |
| Fire C. O. C.              | 510° F.                |
| Pour point                 | 5° F.                  |
| Viscosity at 100° F.       | 380" Saybolt universal |
| Viscosity at 130° F.       | 167" Saybolt universal |
| Viscosity at 210° F.       | 53" Saybolt universal  |
| Viscosity index            | 66                     |
| Color                      | Light 6                |
| Conradson carbon           | 0.20%                  |
| Sulphur                    | 0.45%                  |
| Viscosity gravity constant | .885                   |

This oil, it may be noted, has an unusually good pour, a viscosity index of the same nature as Mid-Continent base lubricants, which is considerably better than Coastal lubricants, and a viscosity-gravity constant which is of acceptable nature. In other respects it is definitely of comparable quality with normal lubricants.

Former attempts to produce lubricants from pressure tar have not resulted in usable lubricant oils, for the reasons pointed out heretofore. The selective solvent treatment of lubricants as heretofore developed has been engaged in bettering the quality of oils already acceptable to a salable degree as lubricants. I am not aware of any indication in the selective solvent treatment of lubricants that would point out that the treatment of a pressure tar fraction by those methods would result in the production of a good lubricant from an oil initially so low in viscosity index, so highly susceptible to oxidation and so high in carbon forming constituents. This is most forcibly pointed out by the unusual increase in viscosity index.

It has not been previously recognized, so far as I am aware, that the cracking of gas oil produces a substantial proportion of products of polymerization which are highly "paraffinic" in nature and capable of being isolated and refined to produce lubricants of the same character as those which might be produced from the heavier fractions of the crude by processes which are at pains to avoid cracking.

My process enables me to recover from pressure still residues a lubricant having a viscosity index of about the same value as Mid-Continent oils, a good viscosity-gravity constant, good resistance to oxidation, and other qualities in every way comparable to regular lubricants, and that in economic percentages. Inasmuch as the source of this oil was originally a gas oil, I have been enabled to materially add to the amount of good lubricants recoverable from a given crude.

Broadly, my process contemplates the treatment of pressure tar by distillation under vacuum, and the refining of the distillate by fractional solution methods, followed by such other conventional operations of dewaxing, etc. as may be found necessary, and it is not intended that it be limited to the conditions which are herein set forth in an exemplary manner only, but only to such limitations as may be found in the appended claims.

What is claimed is:

1. The method of synthesizing a lubricant oil of high viscosity index and resistant to oxidation which comprises the steps of cracking a

gas oil to produce gasoline, cycle gas oil and pressure tar, separating the pressure tar from the remaining products of the cracking operation, subjecting the pressure tar to a non-cracking distillation to produce a non-viscous distillate, a viscous distillate, and a residue, treating the viscous distillate with a selective solvent capable of removing therefrom the portion highly susceptible to loss of viscosity upon rise of temperature, and finishing the remainder of the viscous distillate as a lubricant substantially equal in quality to current lubricants of Mid-Continent origin.

2. In the process of preparing a lubricant oil of high viscosity index and resistant to oxidation from the liquid residue of cracking, the steps which comprise subjecting the liquid residue to non-cracking distillation to produce a non-viscous distillate, a viscous distillate, and a residue, and treating the viscous distillate to remove from it ingredients highly susceptible to loss of viscosity upon rise of temperature, by extraction with liquid sulphur dioxide at low temperature, said treatment being continued until attainment of a raffinate oil having a viscosity index not less than 65 when dewaxed.

3. In the process of preparing a lubricant oil of high viscosity index and resistant to oxidation from the liquid residue of cracking, the steps which comprise subjecting the liquid residue to non-cracking distillation to produce a non-viscous distillate, a viscous distillate, and a residue,

and treating the viscous distillate at low temperature with liquid sulphur dioxide to remove from it ingredients highly susceptible to loss of viscosity upon rise of temperature, thereby to produce a final lubricant product substantially equal in quality to current lubricants of Mid-Continent origin.

4. In the process of synthesizing from petroleum distillates initially containing substantially no fractions of high viscosity a lubricant oil substantially similar in resistance to loss of viscosity with rise in temperature, low carbon content, and resistance to oxidation to lubricant oils of like viscosity normally prepared directly from the viscous fractions of Mid-Continent crude oils, the steps which comprise subjecting the non-viscous petroleum distillate to cracking conditions of temperature and pressure capable of producing therefrom a commercially acceptable yield of gasoline, segregating a liquid residue from the cracking operation which is of higher boiling range than the distillate initially treated, subjecting this liquid residue to distillation under non-cracking conditions of temperature and pressure, collecting the viscous fractions of the distillate so produced, separating from such viscous distillate a portion having low susceptibility to loss of viscosity with rise in temperature by treatment of said oil with liquid sulphur dioxide, and dewaxing the said separated fraction. 30

LESLIE C. BEARD, JR.